

# UNITED STATES PATENT OFFICE.

THOMAS PARKER, OF LONDON, ENGLAND.

## PRODUCTION OF FUEL.

958,761.

Specification of Letters Patent. Patented May 24, 1910.

No Drawing.

Application filed July 29, 1907. Serial No. 386,088.

*To all whom it may concern:*

Be it known that I, THOMAS PARKER, M. I. C. E., a subject of the King of Great Britain and Ireland, residing at 1<sup>st</sup> Chapel 5 street, Edgware Road, London W., England, have invented certain new and useful Improvements in and Relating to the Production of Fuel, of which the following is a specification.

10 This invention relates to the production by partial destructive distillation from coal of a partially coked fuel of high calorific value which in combustion in an open grate shall be practically smokeless and is particularly applicable to the process described 15 in the prior application for Patent No. 354319/07. In the distillation of coal for the production of such a smokeless partially coked fuel I have experienced difficulty in 20 effecting complete gasification of the coal and in the production of a homogeneous partially coked fuel by reason of the caking of the coal near the surface during the process of distillation which causes not only 25 the splitting of the coal and the formation of fissures within it but also prevents the outlet of the gas from within the fuel and thus renders difficult the production of a smokeless partially coked fuel of uniform 30 character and homogeneity. Now according to the present invention I avoid this serious difficulty by applying heat in the process of distillation according to the prior application for Patent No. 354319/07 gradually 35 and slowly so that the process of distillation may first take place at the surface of the coal with such effect as to render the coal at its surface porous and so that thus the process of distillation may then continue 40 by gradual penetration inwardly and that thereby an outlet may be afforded for the liberation of the gases as they are generated within the coal and thus the coal may then be uniformly though partially destructively 45 distilled at a final temperature of about 800° F.

It will be understood that the application of heat to the coal in the process is arrested at that stage when illuminating gas ceases 50 to come off and when the presence of hydrogen and nonluminous gas is indicated by the characteristic flame. By thus arresting the

process of distillation when practically all the illuminating gas has been driven off, a partially coked fuel results which can readily 55 be ignited and which burns freely in an open grate without smoke, its combustion being such as to develop a very high temperature that contributes to this result.

It will be understood that at the commencement of the process the heat applied is slight and that it is very gradually raised so that the whole mass of coal under treatment may be uniformly heated and the heat is gradually and slowly increased for the 60 purpose stated.

I may employ any suitable means for controlling the application of heat to the fuel.

It will furthermore be understood that the invention involves the use of the process the 70 subject-matter of the prior application for Patent No. 354319/07 and that it is also one of the objects of the present invention in addition to obtaining smokeless partially coked fuel, to produce an illuminating gas of high 75 illuminating power as well as other valuable by-products such as tar, and ammonia which render the process of production of the fuel as hereinbefore described highly economical.

It will be also understood that after the 80 partial destructive distillation has been completed, and for the purpose of cooling the fuel and preventing its combustion in air I employ steam superheated or at normal temperature and pressure as in the process of 85 the prior application referred to.

What I do claim as my invention and desire to secure by Letters Patent is:—

In a process for the destructive distillation of coal the application of heat to the 90 retort charged with the coal to be treated, gradually and slowly, up to a maximum ultimate temperature of 800° F. and the arrestment of the process at the stage when illuminating gases have ceased to be evolved, for 95 the purpose and substantially as described.

In testimony whereof I have hereunto signed my name to this specification in the presence of two subscribing witnesses.

THOMAS PARKER.

Witnesses:

RICHARD WILLIAM DAVIES,  
G. Y. WARREN.